

## UNITED STATES PATENT OFFICE

WILFORD BACON HOGGATT, OF NEW LONDON, CONNECTICUT

WATERPROOF AND FIREPROOF FIBROUS PRODUCT AND PROCESS OF MAKING THE  
SAME

No Drawing.

Application filed March 31, 1930. Serial No. 440,633.

This invention relates to combined waterproof and fireproof fibrous products and a process of making the same.

The object of the invention is to produce in a simple and inexpensive manner a non-inflammable water-proof fibrous product.

The invention consists in the combined fireproof and waterproof fibrous product, and process of making the same, all as will be more fully hereinafter set forth, and finally pointed out in the appended claims.

Heretofore various attempts have been made to produce fibrous products, such as pulp boards, panels, and similar articles which are not only waterproof but are also non-inflammable or fireproof, but such efforts have not been attended with any great degree of success for the reason that the materials essential for rendering the products fire-resistant, and those for rendering it water-resistant, when brought together react against each other and impair or destroy their respective fireproofing and waterproofing qualities. Moreover, the methods heretofore suggested for waterproofing and fireproofing the same body or product have been complicated and expensive and have failed to secure the desired degree of efficiency of either the fireproofing or the waterproofing result.

It is among the special purposes of my present invention to provide a fibrous or pulp board, panel or other product, and a process of preparing and making the same, which is not only simple and inexpensive, but in which the combined qualities of fireproofing and waterproofing are most efficiently attained.

In carrying out my invention I propose to employ as the base material for the board, panel or other product any suitable fibrous material, such as wood pulp, cotton linters, fabric, rags, paper, bagasse, cornstalks, or other pulp body of a cellulose fibre character. This base material or pulp is formed in any suitable or well known manner into a board,

panel or other desired product, and either while forming the same into shape, or afterwards, or even while reducing the base material to pulp condition, I apply thereto the required chemicals or materials to render the same both fire-resistant and water-resistant, according to the nature of pulp employed, and in such manner, and by the use of such materials as will enable the particles composing the fibrous body to be thoroughly impregnated with the fireproofing compound, throughout the entire body thereof, and the impregnated particles to be covered or coated with a thin film of the waterproofing compound employed, which does not injure or impair and, in turn, is not injured or impaired by the fireproofing compound.

For securing the desired fireproofing quality of the fibrous board, panel or other product, I prefer to employ a solution containing borax, boracic acid, sulphate of ammonia, and a suitable glue, such as animal glue, ground or flaked, casein, soya bean glue, or the like.

For securing the desired waterproofing quality I propose to employ any suitable waterproofing compound or substance which is soluble in a volatile hydrocarbon such as gasoline, naphtha, benzol, alcohol, or the like. I have found a waterproofing material consisting of wax, either mineral or vegetable, such as paraffin, shale wax, beeswax, Montan wax, or the like, or a combination of resin and wax tailings efficient for my purposes.

It is important to employ a fibrous material for the base or body of the article to be produced, and also a fireproofing compound which will not be attacked or injured by the hydrocarbon solvent for the waterproofing compound.

In preparing the fireproofing compound, and by way of an illustrative example, I take 800 parts by weight of sulphate of ammonia having a nitrogen content of, say, 23% to 25%, 200 parts of borax, 300 parts of boracic

acid, and 350 parts of the desired glue, animal or vegetable, as above stated. The glue is soaked in water, say for eight to twelve hours, or over night, and the ammonia, borax and boracic acid are then added in the proportion of about one gallon of water to 1.65 pounds of the chemicals used. The mass is then thoroughly stirred and mixed at a temperature sufficient to fuse the borax and boracic acid, say at a temperature of about 185° F., more or less. If desired, depending on the nature or character of the fibre employed for the base material, the fireproofing compound, prepared as above explained, may be diluted by adding water thereto.

When the fibrous material, wood, fabric, paper, bagasse, or the like, is reduced to the condition of pulp by grinding, in beaters, or otherwise, in the usual or well known way, the fireproofing compound, prepared as above described, may be employed in place of water or other liquid employed in connection with such grinding or beating. When applied and used in this manner the fireproofing compound becomes thoroughly incorporated into and throughout the body of the fibre base, and serves as a sizer therefor. The pulped material, whether pulped in the presence of the fireproofing compound or not is formed into a board, sheet, panel, or other article to be produced, in the usual or any well known manner, and is then dried. If the pulping operation has been effected with the fireproofing compound, the salts of such compound become uniformly and thoroughly distributed throughout the pulp body, and thoroughly impregnated therein so as to render such body non-inflammable when dried. Excessive temperatures should be avoided in drying the pulp body, the lowest possible drying temperature consistent with speed of output and commercial cost being used. I have found a drying temperature of approximately 180° F. or higher gives good results.

By employing a comparatively low drying temperature the fireproofing chemicals employed become more firmly adherent to the fibre of the base body, the crystallization thereof is reduced to a finer degree, and the glue content is less injured, and retains and imparts greater adhesiveness and hence greater homogeneity to the base body. The product should be removed from the drier as soon as the drying is completed.

While my invention contemplates and includes the pulping of the fibre in the fireproofing compound, and then drying, or partially drying the product, I prefer to first comminute or pulp the fibrous material with water and form it into a sheet or board, or other article and dry, or partially dry it, and then apply the fireproofing compound. In this case the fireproofing compound may be applied either by spraying the same onto the dried board, sheet or article, or impregnated

into the fibre body by the action of a vacuum, or by both, or immersion of the article into the said compound. The important feature is to secure a thorough and uniform penetration of the fireproofing compound into, and distribution of the same throughout the entire fibrous body. Where the compound is applied by means of a vacuum action the surface of the board or sheet is more or less roughened but this is advantageous as it facilitates the penetration of the compound into the body of the fibre base. As the moisture which is retained within the body of the base fibre tends to more or less dilute the fireproofing compound when impregnated into the body, it is preferable to remove more or less of the moisture of the body before spraying, dipping, or immersing the same with or in the compound. If the pulp sheet or board is formed in the usual way by means of vacuum or suction rolls, the application of the fireproofing compound may be effected at any desired point in the board or sheet forming operation, whether such application is effected by spraying, dipping, or immersion, or by vacuumizing.

Where the fibrous material is pulped with the fireproofing compound any desired anti-foaming agent or mixture may be employed. Kerosene is suitable for this purpose, but should be used sparingly in order to avoid damage or injury to the fibre or to the fireproofing quality of the compound.

After the board, sheet or other article has been completed and dried with the fireproofing compound impregnated therein, as above described, the waterproofing composition is then applied. This composition consisting of wax, either mineral or vegetable, such as paraffin, shale wax, Montan wax, beeswax, resin, wax tailings, or the like, dissolved in a hydrocarbon solvent, such for example as gasoline, naphtha, benzol, alcohol, or the like, may be caused to penetrate into the body of the fibrous fireproofed article in various ways. I have found it satisfactory to simply immerse the article in the solution, or to impregnate the article with the solution by means of a vacuum. The naphtha, benzol, alcohol, or other solvent carrier, particularly gasoline, is exceedingly penetrating, not into the fibre particles themselves but around and in enveloping relation with respect to the fibre particles to and into which the fireproofing compound has been applied. The hydrocarbon solvent for the waterproofing compound, however, does not attack nor impair the fibre of the article for the reason that the fibre particles are already protected by the fireproofing material applied thereto which is not affected by the hydrocarbon carrier.

The evaporation of the solvent carrier for the waterproofing solution leaves the waterproofing material as a deposit of a thin film on and around the surfaces of the fibre par-

ticles of the body. This depositing and filming action takes place throughout the entire body of the article being treated, and is a most important feature of my invention as it secures a most efficient waterproofing of a fireproofed fibrous body, a result which, so far as I am aware has never been successfully and satisfactorily accomplished in an economical manner. And in addition fixes the fireproofing chemicals in the body and prevents exudation of the fireproofing salts.

If desired the solvent for the waterproofing material may be recovered for use over again by condensing the vapors given off by the evaporation thereof.

If desired, and in order to increase the adhesion of the fibres in the board or other article, and to strengthen such article, alum or silicate of soda, or both, may be added to the mass during the pulping operation.

Having now set forth the object and nature of my invention and the manner of carrying out the same, what I claim as new and useful and of my own invention is:

25 1. The method of making a fireproofed and waterproofed fibrous article which consists in pulping fibrous material and forming the same into the article to be produced, impregnating such article with a fireproofing compound, drying the article and finally penetrating the fireproofed article with a waterproofing material.

25 2. The method which consists in pulping suitable fibrous material and impregnating the same with a fireproofing compound, drying the fibrous material and finally depositing a film of waterproofing material upon the surfaces of the fireproofed particles of fibrous material throughout the fibrous body.

40 3. The method which consists in pulping suitable fibrous material and impregnating the same with a fireproofing compound, drying said material and finally penetrating the body of the fireproofed fibrous material with a waterproofing compound carried in a volatile solvent, whereby a film of waterproofing material is applied to the surfaces of the particles of fibre of the body.

45 4. The method which consists in pulping suitable fibrous material and impregnating the same with a fireproofing compound, drying said material and finally penetrating the body of the fireproofed fibrous material with a waterproofing substance carried in a hydrocarbon solvent to deposit a film of waterproofing material upon the fireproofed fibrous particles throughout such body.

5. The method which consists in pulping suitable fibrous material and impregnating the same with a fireproofing compound, drying the material and finally penetrating the body of the fireproofed fibrous material with a waterproofing substance carried in solution in gasoline, to deposit a film of waterproofing

material upon the surfaces of the fireproofed fibrous particles throughout such body.

6. The method which consists in pulping suitable fibrous material and impregnating the same with an aqueous compound of sulphate of ammonia, borax, boracic acid, and glue, drying the material and then penetrating the resulting body with a waterproofing material carried in a volatile solvent.

7. The method which consists in pulping suitable fibrous material and impregnating the same with an aqueous compound of sulphate of ammonia, borax, boracic acid, and glue, drying the material and then penetrating the resulting body with a waterproofing material carried in a hydrocarbon solvent.

8. The method which consists in pulping suitable fibrous material and impregnating the same with an aqueous compound of sulphate of ammonia, borax, boracic acid, and glue, drying the material and then penetrating the resulting body with a waterproofing material carried in gasoline.

9. The method which consists in pulping suitable fibrous material and impregnating the same with an aqueous compound of sulphate of ammonia, borax, boracic acid, and glue, drying the material and then penetrating the resulting body with a wax dissolved in a volatile solvent.

10. The method which consists in pulping suitable fibrous material and impregnating the same with an aqueous compound of sulphate of ammonia, borax, boracic acid, and glue, drying the material and then penetrating the resulting body with a wax dissolved in a hydrocarbon solvent.

11. The method which consists in pulping suitable fibrous material and impregnating the same with an aqueous compound of sulphate of ammonia, borax, boracic acid, and glue, drying the material and then penetrating the resulting body with a wax dissolved in gasoline.

12. The method which consists in pulping suitable fibrous material and forming the same into a sheet, and drying it, then impregnating the sheet throughout with a fireproofing compound, drying the sheet again and finally penetrating the fireproofed sheet with a waterproofing material.

13. The method which consists in pulping suitable fibrous material and forming the same into a sheet, and drying it, then impregnating the sheet throughout with a fireproofing compound, drying the sheet again and finally penetrating the fireproofed sheet with a wax.

14. The method which consists in pulping suitable fibrous material and forming the same into a sheet, and drying it, then impregnating the sheet throughout with a fireproofing compound, drying the sheet again

70

75

80

85

90

95

100

105

110

115

120

125

130

and finally penetrating the fireproofed sheet with paraffin carried in a volatile solvent.

15. The method which consists in pulping suitable fibrous material and forming the same into a sheet, and drying it, then impregnating the sheet throughout with a fireproofing compound, drying the sheet again and finally penetrating the fireproofed sheet with paraffin dissolved in gasoline.

10 In testimony whereof I have hereunto set my hand on this 12th day of March, A. D. 1930.

WILFORD BACON HOGGATT.

15

20

25

30

35

40

45

50

55

60

65